

## UNITED STATES PATENT OFFICE

SAMUEL S. SADTLER, OF SPRINGFIELD TOWNSHIP, MONTGOMERY COUNTY, AND EUGENE F. CAYO, OF PHILADELPHIA, PENNSYLVANIA, ASSIGNOR TO AMIESITE ASPHALT COMPANY OF AMERICA, OF PHILADELPHIA, PENNSYLVANIA, A CORPORATION OF NEW JERSEY

## ROAD COMPOSITION

No Drawing. Application filed September 15, 1926. Serial No. 135,702.

This invention relates to roads, and particularly to road compositions comprising asphalt or other bitumen with a rock aggregate, and the principal object of the invention is to provide a novel method for forming a bitumen road composition using an undried or wet aggregate, whereby the expensive drying operation normally required in order to effect a close bond between the aggregate and the bitumen may be eliminated.

In the building of roads of this type, the stone aggregate invariably is received in a damp and often wet condition, and although in certain types of road stone in this condition has been mixed with asphalt or other bitumen, roads so made lack cohesion and close union between the aggregate and the bitumen and are therefore unstable. It accordingly is customary in making the better grades of road and road compositions to dry the aggregate and to free it of all or the greater part of its moisture content.

In one type of road it also is highly desirable to obtain in the stone aggregate an absorption and storage of an appreciable amount of a bitumen solvent, this having among other desirable effects that of rendering the curing process of the finished road a comparatively slow one. The use of damp or wet stone as ordinarily used positively precludes the possibility of getting this desirable storage effect, and this fact has resulted again in a requirement for an extensive preliminary drying of the aggregate.

It is the principal object of this invention therefore to provide a commercially practicable method for obtaining a thorough bond between the aggregate and the bitumen without a predrying operation regardless of the amount of moisture present, and also under similar conditions to obtain, where desired, the aforesaid storage in the aggregate of a bitumen solvent.

In carrying out our invention, we preferably thoroughly wash the stone aggregate by spraying with warm water, this having the multiple effect of cleaning out the fines and dust, bringing the entire aggregate to a uniform condition of wetness, and raising the temperature of the wet stone to a moderate

temperature of say 95° F. In some instances, it may be desirable to retain the fines, and in such cases provision may be made either for preventing their removal or for reincorporating them in the aggregate.

We then take the wet and preferably warm stone and thoroughly mix with it by any suitable means a quantity of a soluble soap, such for example as saponified sulfonated oil, or any commercial soap, which may be incorporated either in a powdered and dry condition, or in liquid form. The quantity of soap employed may vary widely, although we have found satisfactory, approximately one pound of the soap to each ton of aggregate. When this soap has been thoroughly incorporated and mixed with the aggregate, we add a quantity of a more or less volatile bitumen solvent, such as kerosene, gasoline or the like, and agitate the mass. The quantity of this solvent may vary largely, although for general purposes about two gallons per ton of aggregate will be found sufficient. This solvent forms with the water and the soluble soap an emulsion of the oil-in-water type, in which the water is the continuous element, and we thereby replace the water in the interstices and pores of the stone and on the surface thereof with the water and oil emulsion. This in general has the effect of replacing the water in and on the stone with emulsion, the water particles, however, being in continuous phase.

The aggregate is now in condition to receive the asphalt or other bitumen binder, and this we may now add in sufficient quantity to thoroughly coat the individual stones. A normally solid asphalt is used, and for this mixing operation we temporarily liquefy the asphalt, preferably by heating; a temperature of about 240° F. is preferred. Although it is preferred to use heat as the liquefying agent, the desired result may be effected by other means, as by adding to the bitumen a suitable volatile solvent or liquefier such as gasoline. Where a solvent is used as the liquefying agent, the solvents originally added to the aggregate may be dispensed with. In this event, however, at least a part of the solvent or liquefier used preferably is

of a slowly volatile character, such as kerosene.

We now preferably add to the mass lime or lime-containing material, or in fact any material having a suitably high content of alkaline-earth preferably in not too soluble form, in proportionate amount approximately eight pounds per ton batch of stone. This substance has the desirable effect of slowly 10 setting the soap and producing a calcium soap which is insoluble, and insuring alkaline reaction in the composition. The water, freed from the emulsion, separates from the mass soon after the lime is added.

15 As an actual preferred example of our process, we may take 1900 pounds of wet stone aggregate free from fines and dust and preferably at a temperature of about 95° F., and add thereto approximately one pound 20 of saponified sulfonated oil, thoroughly mixing and incorporating this soap in the aggregate. We now add about two gallons of approximately 50% mixture of kerosene and naphtha, and following the mixing in of 25 these solvents, we add to the aggregate asphalt in amount to thoroughly coat the individual stones, the asphalt being in fluid state and at a temperature of about 240° F., and rapidly incorporate it by stirring. Generally, asphalt in amount equal to 5% by 30 weight of the aggregate will be sufficient. Thereafter, we preferably add lime in amount approximately eight pounds per ton batch of the bitumen-stone composition.

35 By this process we are able to provide an asphaltic road in which the individual stones are thickly and with substantial permanency coated with the bitumen. The aggregate also retains in temporary storage an appreciable amount of the kerosene, retarding 40 the final set of the composition after it has been laid upon the roadbed. Of primary importance, however, the process provides for the use of wet stone in the manufacture of 45 bitumen road compositions without special drying operations, and thereby creates a material saving.

It will be understood that the process may be varied to some extent from that outlined 50 above without departure from the invention. It is possible for example as suggested above to add the bitumen solvent and the bitumen simultaneously either individually or in the form of a mixture previously prepared. In 55 fact, the benefits of the invention may be realized to some extent by adding the bitumen in advance of the liquefier. There may also be some variation as to the addition of the emulsifying agent, since it is not strictly essential that this be added directly to the wet stone in advance of the other elements. There also is to be no strict limitation as to 60 the relative proportions of the various materials used, since these also may vary in large degree. The procedure and proportions de-

tailed in the specification, however, have been found satisfactory and are preferred.

We claim:

1. The method of forming a road composition, which consists in taking a stone aggregate in moist condition and mixing therewith a bitumen solvent, an agent adapted to form an oil-in-water emulsion with the said solvent and the moisture content of the stone, lime, and a temporarily liquefied bitumen. 70

2. The method of forming a road composition, which consists in mixing with a stone aggregate in moist condition and in any sequence or order a bitumen solvent including 80 kerosene, an agent adapted to form an oil-in-water emulsion with the said solvent and the moisture content of the stone, and a temporarily liquefied bitumen, and when the aggregate is coated with said ingredients adding 85 to the mixture an ingredient operative to break the emulsion.

3. The method of forming a road composition, which consists in mixing with a stone aggregate in moist condition and in any order or sequence a bitumen solvent consisting 90 of a 50% mixture of kerosene and naphtha, an agent adapted to form an oil-in-water emulsion with the said solvent and the moisture content of the stone, and a temporarily liquefied bitumen, and subsequently adding 95 an alkaline earth ingredient to break the emulsion.

4. The method of forming a road composition, which consists in adding directly to 100 a stone aggregate in moist condition an agent adapted to form an oil-in-water emulsion with a subsequently added solvent of bitumen and the moisture content of the stone, and thereafter adding the said solvent, and a temporarily liquefied bitumen, and subsequently adding an ingredient to slowly break the emulsion. 105

5. The method of forming a road composition, which consists in adding directly to 110 a stone aggregate in moist condition an agent adapted to form an oil-in-water emulsion with a subsequently added solvent of bitumen and the moisture content of the stone, thereafter adding the said solvent, and a 115 temporarily liquefied bitumen, and subsequently adding an alkaline earth ingredient operative to slowly break said emulsion.

6. The method according to claim 1, in which the elements employed are proportionately as follows: stone aggregate 1900 lbs., bitumen 100 lbs. of asphalt, solvent 1 to 2 gallons of a 50% mixture of kerosene and naphtha, emulsifying agent 1 lb. of saponified sulfonated oil, and 6 to 10 lbs. of lime. 120

7. The method of forming a road composition, which consists in mixing with a mineral aggregate in a moist condition and in any sequence or order, a bitumen solvent, an agent adapted to form an oil in water emulsion 130

with said solvent and the moisture content of said aggregate, and a temporarily liquefied bitumen, and subsequently adding thereto an ingredient operative to break said emulsion.

8. The method of forming a road composition, which consists in mixing with a mineral aggregate in a moist condition, a bitumen solvent, a water-soluble soap adapted to form an oil in water emulsion with said solvent and the moisture content of the aggregate, and a temporarily liquefied bitumen, and thereafter adding to the mixture, an agent operative to convert said water-soluble soap into a water-insoluble soap.

SAMUEL S. SADTLER.  
EUGENE F. CAYO.

20

25

30

35

40

45

50

55

60

65